# EUROPEAN PATENT SPECIFICATION

(11) **EP 0 086 444 B1**
(45) Date of publication and mention of the grant of the patent: **20.05.1987**
(21) Application number: 83101193.7
(22) Date of filing: 08.02.1983
(51) Int. Cl.: H01F 1/36, G03G 9/10, C04B 35/26

(54) **Magnetic carrier powder for two-component toner**
Magnetisches Pulver für Zweikomponenten-Toner
Poudre magnétique pour toner à deux composants

(30) Priority: 13.02.1982 JP 21923/82
(43) Date of publication of application: 24.08.1983
(73) Proprietor: TDK Corporation, Chuo-ku, Tokyo-to 103 (JP)
(72) Inventor: Imamura, Kenji, c/o TDK Electronics Co. Ltd., Chuo-ku, Tokyo 103 (JP); Saitoh, Hiroshi, c/o TDK Electronics Co. Ltd., Chuo-ku, Tokyo 103 (JP); Kakizaki, Katsuhisa, c/o TDK Electronics Co. Ltd., Chuo-ku, Tokyo 103 (JP); Makino, Motohiko, c/o TDK Electronics Co. Ltd., Chuo-ku, Tokyo 103 (JP)
(74) Representative: Wächtershäuser, Günter, Prof. Dr.

## Description

The present invention relates to a magnetic brush development magnetic carrier powder.

Heretofore, as a magnetic carrier powder to be used for magnetic brush development, there has been used an iron powder or a soft ferrite powder and it has been believed that the average particle size of the powder should preferably be from 30 to 1000 pm.

However, such a conventional carrier powder is not totally satisfactory in that it does not provide satisfactory image quality such as a resolving power, graininess, black uniformity or gradation of the image.

A different type of magnetic toner powder is described in EP-A-10 732. The ferrite powder type magnetic toner of this reference comprises ferrite particles having a spinel structure incorporated in a resinous component.

Under these circumstances, it is the primary object of the present invention to provide a magnetic carrier powder which is capable of providing an image having an improved image quality such as the resolving power, graininess, black uniformity or gradation.

The present inventors have conducted extensive researches and as a result, have found that the object can be attained by reducing the ferrite powder particles to have an average particle size smaller than that of the conventional ferrite particles. Namely, the present invention provides a magnetic brush development magnetic carrier powder composed of ferrite powder particles having a spinel structure and an average particle size of from 5 to 30 pm, said powder particles not having a coating layer and not being incorporated in a resin.

There has hitherto been no instance where ferrite powder particles having such a small particle size have been used alone as a carrier.

Now, the present invention will be described in detail with reference to the preferred embodiments.

The magnetic carrier powder of the present invention is made of a ferrite having a spiral structure.

As the ferrite having a spinel structure, there may be mentioned a so-called soft ferrite such as a 2-3 spinel or a 1-3 spinel, a magnetite (Fe₃0₄) or a maghemite (y-Fe₂0₃).

Among these ferrites, the following ferrites i) and ii) are particularly preferred in view of its magnetic characteristics.

i) a spinel ferrite comprising at most 60 molar % of MO where M is Ni, Mn, Mg, Zn, Cu, Co or a combination thereof, as calculated as a divalent oxide, and at least 40 molar % of Fe₂0₃ as calculated as a trivalent metal oxide.

In this case, where M is a combination of at least two kinds of metals, their proportions may be optionally selected.

ii) a magnetite.

Among the ferrites i), the following ferrites ia) and ib) are preferred.
ia) a ferrite i) wherein M is Ni, Mn, Mg, Cu, Zn or a combination thereof. In this case, when M is a combination of at least two kinds of metals, their proportions may be optionally selected.
ib) a ferrite i) wherein M is a combination of Ni, Mn, Mg, Cu, Zn or a combination thereof, with at most 20 atom % of Co. In this case, when M is a combination of at least two kinds of metals selected from Ni, Mn, Mg, Cu and Zn, their proportions may be optionally selected.

When such a ferrite ia) or ib) is used, the saturation magnetization becomes extremely high, whereby the deposition of the carrier on the photosensitive material or scattering of the carrier from the magnetic brush can be minimized.

The ferrite powder particles having the above-mentioned composition may further contain at most 5 molar % of an oxide of Ca, Bi, Cr, Ta, Mo, Si, V, B, Pb, K, Na, or Ba.

Such ferrite powder particles have an average particle size of less than 30 !-1m.

If the average particle size is 30 pm or greater, the image quality, particularly the resolving power, graininess, uniformity or gradation tends to be degraded. Further, the image quality tends to be of high contrast, which taxes the eyes of the observer.

On the other hand, if the average particle size is too small, the deposition of the carrier particles on the photosensitive material or the scattering of the carrier tends to be pronounced and the flowability of the developer tends to be poor. Therefore, the average particle size should preferably be at least 5 pm. Particularly good results are obtainable when the average particle size is from 5 to 25 pm.

Further, the particle size distribution is usually such that about 70% of the total particles have a particle size falling within the range of ±30% of the average particle size.

Such ferrite particles are used as a carrier without being coated with a coating layer on the surfaces or without being dispersed in a resin. Therefore, the magnetic carrier powder of the present invention has great mechanical strength and hardly undergoes thermal degradation, whereby the degradation of its properties with time is minimum and its useful life is very long. Further, the reduction of the saturation magnetization due to the decrease of the volume occupying rate is minimum and its production is quite easy.

The ferrite powder particles constituting the magnetic carrier powder of the present invention preferably have an electric resistance of from 10⁴ to 10¹⁴ Ω, more preferably from 10⁵ to 10¹²Ω, when 100 V is applied in the following manner.

Namely, the measurement of the electric resistance of the ferrite powder particles is conducted in the following manner in accordance with a magnetic brush development system. An N-pole and a S-pole are arranged to face each other with a magnetic pole distance of 8 mm so that the surface magnetic flux density of the magnetic poles becomes 0.15 tesla (1500 Gauss) and the surface area of the facing poles is 10x30 mm. Between the magnetic poles, a pair of flat non-magnetic electrodes are disposed in parallel to each other with an electrode distance of 8 mm. Between the electrodes, 200 mg of a test sample is placed and the sample is held between the electrodes by the magnetic force. With this arrangement, the electric resistance is measured by an insulation resistance tester or an ampere meter.

If the electric resistance as measured in such a manner exceeds 10¹⁴ Q, the image density tends to be low. On the other hand, if the resistance is less than 1040, the image quality tends to be of high contrast.

Further, in the present invention, the saturation magnetization σₘ of the ferrite particles is preferably at least 35 emp/g, whereby the deposition of the carrier on the photosensitive material or the scattering of the carrier by repeated development operations can be minimized. In this case, better results are obtainable when the saturation magnetization aₘ is at least 40 emµ/g.

The magnetic carrier powder composed of such ferrite powder particles may be prepared in such a manner as disclosed in U.S. Patent No. 3,839,029, No. 3,914,181 or No. 3,929,657.

Namely, firstly, the corresponding metal oxides are mixed. Then, a solvent such as water is added and the mixture is slurried, for instance, in a ball mill. Other additives such as a dispersing agent and a binder may be added as the case requires. Then, the slurry is granulated and dried by a spray drier. Thereafter, the granules thereby obtained are burned at a predetermined burning temperature in a predetermined burning atmosphere. The burning is conducted in a fluidized furnace, a rotary kiln or a tunnel furnace, whereby particles having the above-mentioned average particle size is efficiently produced. After the burning, the particles are pulverized or dispersed to obtain a desired particles size, whereby the magnetic carrier powder of the present invention is obtained.

The magnetic carrier powder of the present invention is mixed with a toner to obtain a developer. In this case, the type of the toner to be used is not critical and any toner may be used. Further, the magnetic brush development system and the photosensitive material to be employed to obtain an electrostatic copy image are not critical and an electrostatic copy image can be obtained in accordance with a conventional magnetic brush development method.

According to the present invention, an extremely good image quality is obtainable. Namely, the resolving power, graininess, black uniformity and gradation thereby obtained are extremely good. The image is of soft gradation, which does not very much tax the eyes of the observer.

Further, the composition of the ferrite powder particles or the conditions for the burning may readily be varied to optionally change the quantity of magnetism or electric resistance so that images having various image densities and gradations may readily be obtained.

Further, the ferrite powder particles do not having a coating layer or they are not incorporated in a resin. Therefore, the degradation of the characteristics is minimum even when they are used for a long period of time, and they have good durability and a long useful life. They are free from the reduction of the magnetic characteristics which is likely to be led when incorporated with a resin component. Further, the number of the steps for their production can be minimized and the production is easy, whereby the production costs will be low.

Now, the present invention will be described in further detail with reference to Examples. Examples:
Metal oxides were mixed at various ratios (calculated as a divalent metal oxide and Fe₂0₃) as shown in Table 1. One part by weight of water was added to one part by weight of each mixture and mixed in a ball mill for five hours to obtain a slurry. Appropriate amounts of a dispersing agent and a binder were added.

Then, the slurry was granulated and dried at a temperature of at least 150°C by a spray drier.

Each granular product was burned in a fluidized furnace at the maximum temperature as shown in Table 1 in the atmosphere also as shown in Table 1. In Table 1, A represents an air atmosphere and N represents a nitrogen atmosphere.

Thereafter, the granules were pulverized and classified to obtain ferrite powder particles having the average particle size as shown in Table 1. The average particle size is an average particle size of 5000 particles randomly selected under observation by an electron microscope. In the Table, the average particle size of 20 pm indicates that the particles have a particle size within a range of from 5 to 30 µm; the average particle size 40 µm indicates that the particles have a particle size within a range of from 25 to 55 µm; and the average particle size of 70 pm indicates that the particles have a particle size within the range of from 40 to 100 pm.

On the other hand, each powder of the ferrite powder particles was subjected to an X-ray analysis, whereby it was confirmed that each powder had a spinel structure and the metal contents corresponding to the feed composition as shown in Table 1.

Then, the saturation magnetization aₘ (emp/g) of each powder of the ferrite powder particles and the electric resistance (Q) under application of 100 V were measured. The results thereby obtained are shown in Table 1. The saturation magnetization am was measured by magnetometer of a sample vibration type. The electric resistance was obtained by measuring electric resistance of the samples of 200 mg by application of 100 V in the aforementioned manner by an insulation resistance meter.

Each ferrite powder thus obtained was used by itself as a magnetic carrier powder. Namely, it was mixed with a commercially available two-component toner (an average particle size of 11.5±1.5 µm) to obtain a developer having a toner concentration of 11.5% by weight.

With use of each developer, magnetic brush development was carried out by means of a commercially available electrostatic copying machine and the image quality of the image thereby obtained was evaluated. In this case, the surface magnetic flux density of the magnetic roller for the magnetic brush development was 0.1 tesla (1000 Gauss); the rotational speed of the magnetic roller was 130 rpm and the rotational speed of the sleeve roller was 30 rpm. Further, the space between the magnet roller and the photosensitive material was 3.0±0.3 mm. As the photosensitive material, a CdS photosensitive material of binder type was used and the maximum surface electric potential was 800 V.

The resolving power (lines/mm) was measured by means of a test chart made by Data Quest Company. The image of the test chart was observed by naked eyes to evaluate the graininess. The evaluation was made in accordance with five ratings A to E where A represents the best and E represents the worst.

Further, the gradation was evaluated by observation with naked eyes. The evaluation was made by means of a grade scale comprising 13 grades and the expressed by the grade numbers (1-13).

The soft gradation was evaluated also by observation with naked eyes. In this case, the order of superiority was expressed by a number.

The results thereby obtained are shown in Table 2.

With each sample, the deposition of the carrier on the photosensitive material and the scattering of the carrier were extremely small.

From the results shown in Table 2, it is evident that the magnetic carrier powders of the present invention give far superior electrostatic images to those having an average particle size of at least 30 pm.

## Claims

1. A magnetic brush development magnetic carrier powder composed of ferrite powder particles having a spinel structure and an average particle size of from 5 to 30 pm, said powder particles not having a coating layer and not being incorporated in a resin.

2. The magnetic carrier powder according to Claim 1 wherein the ferrite powder particles are made of a soft ferrite selected from 2-3 spinel and 1-3 spinel ferrites, a magnetite or a maghemite.

3. The magnetic carrier powder according to Claim 1 wherein the ferrite powder particles are made of a spinel ferrite comprising at most 60 molar % of MO where M is Ni, Mn, Mg, Zn, Cu, Co or a combination of at least two metals thereof, as calculated as a divalent metal oxide, and at least 40 molar % of Fe₂0₃ as calculated as a trivalent metal oxide.

4. The magnetic carrier powder according to Claim 1 wherein the ferrite powder particles are made of a magnetite.

5. The magnetic carrier powder according to Claim 3 wherein M is Ni, Mn, Mg, Cu, Zn or a combination thereof.

6. The magnetic carrier powder according to Claim 3 wherein M is Ni, Mn, Mg, Cu, Zn or a combination of at least two metals thereof, with at most 20 atom % of Co.

7. The magnetic carrier powder according to Claim 3 wherein the spinel ferrite contains at most 5 molar % of an oxide of Ca, Bi, Cr, Ta, Mo, Si, V, B, Pb, K, Na or Ba.

8. The magnetic carrier powder according to Claim 1 wherein the average particle size is within a range of from 5 to 25 pm.

9. The magnetic carrier powder according to Claim 1 wherein the ferrite powder particles have a particle size distribution such that at least 70% of the particles have a particle size within a range of ±30% of the average particle size.

10. The magnetic carrier powder according to Claim 1 wherein the ferrite powder particles have an electric resistance of from 10⁴ to 10¹⁴ Q, preferably from 10⁵ to 10¹² Ω, when 100 V is applied.

11. The magnetic carrier powder according to Claim 1 wherein the ferrite powder particles have a saturation magnetization σₘ of at least 35 emp/g.

## Patentansprüche

1. Ein magnetisches Trägerpulver für die magnetische Bürstenentwicklung, zusammengesetzt aus Ferritpulverteilchen mit einer Spinellstruktur und einer durchschnittlichen Teilchengröße von 5 bis 30 pm, wobei die Pulverteilchen keine Beschichtung aufweisen und nicht einem Harz einverleibt sind.

2. Magnetisches Pulver gemäß Anspruch 1, wobei die Ferritpulverteilchen aus einem weichen Ferrit bestehen, ausgewählt aus 2-3-Spinell-_{.}und 1-3-Spinell-Ferriten, einem Magnetit oder einem Maghemit.

3. Magnetisches Pulver gemäß Anspruch 1, wobei die Ferritpulverteilchen aus einem Spinellferrit bestehen, umfassend mindestens 60 Mol-% MO, wobei M für Ni, Mn, Mg, Zn, Cu, Co oder eine Kombination von mindestens zwei dieser Metalle besteht, berechnet als ein zweiwertiges Metalloxid, und mindestens 40 Mol-% Fe₂0₃, berechnet als ein dreiwertiges Metalloxid.

4. Magnetisches Pulver gemäß Anspruch 1, wobei die Ferritpulverteilchen aus einem Magnetit bestehen.

5. Magnetisches Pulver gemäß Anspruch 3, wobei M für Ni, Mn, Mg, Cu, Zn oder eine Kombination derselben steht.

6. Magnetisches Pulver gemäß Anspruch 3, wobei M für Ni, Mn, Mg, Cu, Zn oder eine Kombination von mindestens zwei dieser Metalle steht, mit höchstens 20 Atom-% Co.

7. Magnetisches Pulver gemäß Anspruch 3, wobei der Spinellferrit höchstens 5 Moi-% eines Oxids von Ca, Bi, Cr, Ta, Mo, Si, V, B, Pb, K, Na oder Ba enthält.

8. Magnetisches Pulver gemäß Anspruch 1, wobei die durchschnittliche Teilchengröße in einem Bereich von 5 bis 25 pm liegt.

9. Magnetisches Pulver gemäß Anspruch 1, wobei die Ferritpulverteilchen eine derartige Teilchengrößenverteilung haben, daß mindestens 70% der Teilchen eine Teilchengröße innerhalb eines Bereichs von ±30% der durchschnittlichen Teilchengröße aufweisen.

10. Magnetisches Pulver gemäß Anspruch 1, wobei die Ferritpulverteilchen einen elektrischen Widerstand von 10⁴ bis 10¹⁴ Ω, vorzugsweise von 10⁵ bis 10¹² Ω aufweisen, wenn 100 V angelegt werden.

11. Magnetisches Pulver gemäß Anspruch 1, wobei die Ferritpulverteilchen eine Sättigungsmagnetisierung σₘ von mindestens 35 emµ/g haben.

## Revendications

1. Poudre de support magnétique pour développement au pinceau magnétique composée de particules de poudre de ferrite ayant une structure de spinelle et une dimension de particules moyenne de 5 à 30 µm, ces particules de poudre n'ayant pas de couche de revêtement et n'étant pas incorporées dans une résine.

2. Poudre de support magnétique suivant la revendication 1, caractérisée en ce que les particules de poudre de ferrite sont faites d'une ferrite douce choisie parmi les ferrites de spinelle 2-3 et de spinelle 1-3, les magnétites et les maghémites.

3. Poudre de support magnétique suivant la revendication 1, caractérisée en ce que les particules de poudre de ferrite sont faites d'une ferrite de spinelle comprenant au moins 60 moles % de MO, où M représente Ni, Mn, Mg, Zn, Cu, Co ou une combinaison d'au moins deux de ces métaux, tels que calculés sous la forme d'oxyde métallique bivalent, et au moins 40 moles % de Fe₂0₃ tels que calculés sous la forme d'oxyde métallique trivalent.

4. Poudre de support magnétique suivant la revendication 1, caractérisée en ce que les particules de poudre de ferrite sont faites d'une magnétite.

5. Poudre de support magnétique suivant la revendication 3, caractérisée en ce que M représente Ni, Mn, Mg, Cu, Zn ou une combinaison de ceux-ci.

6. Poudre de support magnétique suivant la revendication 3, caractérisée en ce que M représente Ni, Mn, Mg, Cu, Zn ou une combinaison d'au moins deux de ces métaux, avec tout au plus 20 atomes % de Co.

7. Poudre de support magnétique suivant la revendication 3, caractérisée en ce que la ferrite de spinelle contient tout au plus 5 moles % d'oxyde de Ca, Bi, Cr, Ta, Mo, Si, V, B, Pb, K, Na ou Ba.

8. Poudre de support magnétique suivant la revendication 1, caractérisée en ce que la dimension de particules moyenne est de l'ordre de 5 à 25 µm.

9. Poudre de support magnétique suivant la revendication 1, caractérisée en ce que les particules de poudre de ferrite ont une distribution de dimensions de particules telle qu'au moins 70% des particules ont une dimension de particules de l'ordre de ±30% de la dimension de particules moyenne.

10. Poudre de support magnétique suivant la revendication 1, caractérisée en ce que les particules de poudre de ferrite ont une résistance électrique de 10⁴ à 10¹⁴ Ω, de préférence de 10⁵ à 10¹² Ω, lorsque l'on applique 100 V.

11. Poudre de support magnétique suivant la revendication 1, caractérisée en ce que les particules de poudre de ferrite ont une magnétisation de saturation aₘ d'au moins 35 emµ/g.
